

1

2,893,814

## METHOD OF METALLIZING AZOIC DYEINGS

Clemens Streck, Loudonville, N.Y., assignor to General Aniline & Film Corporation, New York, N.Y., a corporation of Delaware

No Drawing. Application December 28, 1956  
Serial No. 631,062

17 Claims. (Cl. 8—42)

This invention relates to an improved process of metallizing azoic dyeings and particularly to an improved process whereby said dyeings are obtained without the precipitation of free metal on the fibre and dyeing apparatus.

It is known that fibres may be impregnated with a coupling component and passed into a solution which contains an active diazo, either in the form of a freshly prepared diazo or as a fast color salt solution under conditions suitable for coupling. Fast color salts are diazo compounds which, except for a few diazos which are sufficiently stable per se, are diazo compounds which are stabilized by salt formation such as with certain metallic salts, e.g.  $MgCl_2$ ,  $ZnCl_2$ ,  $SnCl_2$ , etc., aryl-sulfonic acids such as naphthalene-1,5-disulfonic acid and naphthalene-1,3,6-trisulfonic acid, and also borofluoric acid.

One of the outstanding advantages of azoic dyeings is their fastness in contrast to that of the usual azo dyes. The fastness of azoic dyeings has recently been improved by metallizing, i.e. by treating the previously dyed fibres with various metallizing agents such as Cu, Co, Cr, Ni and the like. In the art as now practiced, it is necessary to dye the fibrous material with an azoic dye devoid of solubilizing groups followed by an after treatment with a metallizing agent. The metallizing step represents an extra step and also requires at least 20' minutes. To overcome this, satisfactory metallization of azoic dyeings is achieved by incorporating the metallizing agent in the soaping bath as taught in my United States patent application (Serial No. 316,305), now United States Patent 2,768,053.

In my United States patent application Serial No. 601,658, filed on August 2, 1956, for "Method of Metallizing Azoic Dyeings," I disclose and claim a novel process whereby the azoic color formation is carried out in the presence of the metallizing agent. By this process fibrous material dyed with an azoic dye, free from solubilizing groups and capable of conversion into a complex metal compound, is endowed with improved light-, wash- and chlorine-fastness properties and of improved shade. In this process the metallizing agent may be dissolved in a naphtholating bath, the fibrous material impregnated with this bath, usually followed by drying, and the impregnated fibre padded or printed with an active diazo which includes a freshly prepared diazo or a diazo stabilized as a fast color salt, and then metallizing with hot water or preferably with steam. The temperature and moisture conditions of the hot water or steam are sufficiently drastic to yield complete metallization together with color development, even when exposed to steam for less than 1 minute. The important advantage of this improved method is that a satisfactory metallized product is obtained without any additional operations other than the usual dyeing steps. By this procedure, economical dyeings are obtained as contrasted with the present method of after metallizing which requires additional steps, over and above the dyeing steps, i.e., treatment with the metallizing agent and heating.

2

Despite the fact that economical dyeings having desirable characteristics are obtained, the process nevertheless lacks one factor which is highly desirable in the dye trade. In conducting numerous experiments with the process described in the aforesaid application, i.e., Serial No. 601,658, I found that under certain conditions, free copper is precipitated. The precipitation may be on the fibre, causing splotchy dyeings, or in the dyeing apparatus, such as glass, steel, wood, stainless steel, etc. resulting in a metal plating problem. The precipitation is believed to be due to the presence of certain impurities or by-products which are readily oxidizable and in oxidation cause a reduction of the loosely coordinated copper salt to free copper. Cleaning off deposited copper from equipment is difficult in addition to the poor, uneven dyeings resulting therefrom.

I have found that precipitation can be very readily remedied by the addition of an inorganic or organic oxidizing agent to the metallizing solution. The metallizing solution and other details with regard to the diazo and coupling components employed in azoic dyeings are fully described in my aforementioned patent application (Serial No. 601,658), the disclosure of which is incorporated herein by reference thereto. The inorganic and organic oxidizing agents which I have found particularly useful include all of those which are soluble in alkaline aqueous solutions, and are sufficiently stable to withstand the temperature of padding which ranges from room temperature to 212° F., and will not destroy the diazo components. As illustrative examples of such oxidizing agents, the following may be mentioned:

m-Nitrobenzenesulfonic acid  
p-Nitrobenzenesulfonic acid  
Sodium chromate  
Potassium chromate  
Sodium perborate  
Potassium perborate  
Sodium peroxide  
Potassium peroxide  
Hydrogen peroxide

The foregoing oxidizing agents may be present in the amount of about 10-100% based on the weight of the metallizing agent. As stated in my aforementioned patent application, the metallizing agents or compound employed in the metallizing of azoic dyeings are salts and hydroxides of copper (cupric). They are employed in the form of chlorides, sulphates, acetates, formates, nitrates, and the like. Those compounds are preferred which are relatively water soluble or dispersible. The amount of copper salt or copper hydroxide, to be employed will usually depend on the degree of metallizing desired. Molar ratios are necessary for complete metallization but the amount may range from about a fraction of an equivalent to an excess of one equivalent of metal per equivalent of dye. The preferred amount is about 0.5 mol metal salt per mol of dye.

The oxidizing agent may be added to the metallizing solution together with a chelating agent and this solution employed directly to treat the fibre alone or in combination with Naphthol AS compounds which are arylides of 2-hydroxy-3-naphthoic acid and related  $\beta$ -hydroxy carboxylic acid derivatives, acetoacetylides and related  $\beta$ -oxocarboxylic acid arylides and pyrazolones. However, other compounds may be employed which have active methylene or enolizable ketone groups and are free from solubilizing groups such as sulfonic and carboxylic acid groups and which are capable of coupling to yield a component having the required metallizable group in ortho position to the azo linkage, e.g. o-amino-phenol- $\alpha$ -sorcinol.

Instead of employing a combination of the oxidizing

agent, metallizing agent and chelating agent in the treatment, the chelated metallizing agent or oxidizing agent can be combined with a naphtholating solution or Rapidogen solution in the products per se or prior to dyeing and printing. A chelated metallizing agent in dry form and a suitable oxidizing agent can be incorporated in a dry naphthol or Rapidogen powder. Further, the un-coordinated metal salt can be incorporated in a dry naphthol or Rapidogen powder together with suitable oxidizing agent; however such mixture must be pasted with the proper chelating agent prior to use. While the above describes the addition of oxidizing agent to the naphthol or Rapidogen per se, it may be added at any time prior to use. The proportions of chelating agent, metallizing compound, Naphthol AS compound or Rapidogen powder are given in my pending patent application Serial No. 601,658.

In order to practice one embodiment of the present invention, a metallizing solution is first prepared in accordance with the following recipe.

1 to 200 parts of metallizing compound  
5 to 800 parts of water  
1 to 30 parts of chelating agent  
.5 to 80 parts of caustic soda (dry)

After formation of the metallizing solution, 10-100% of an oxidizing agent is added to the solution based on the weight of the metallizing compound.

The following examples will illustrate the preferred embodiments of the present invention. It is to be clearly understood that these examples are illustrative and are not to be considered as limitative.

#### Example I

A metallizing solution containing an oxidizing agent was prepared as follows:

##### Copper solution—

147 grams of copper sulfate  
643 grams of water  
110 grams of triethanolamine  
60 grams of caustic soda (dry)

After formation of a blue solution, 40 grams of sodium chromate anhydrous was added.

A padding solution was prepared by mixing the following components:

3 grams of Naphthol AS (3-hydroxy-2-naphthanolide)  
6 cc. of ethyl alcohol  
1.5 cc. of caustic soda 34° Bé.

The padding solution was poured into 10 cc. of the above copper solution together with 2.5 cc. of caustic soda 34° Bé. and water to yield a total volume of 133 cc.

A 10 gram sample of muslin was padded with the above solution, dried and padded with a solution consisting of:

7 grams of o-dianisidine, tetrazotized and stabilized with zinc chloride,  
.5 cc. of Diazopon AN (fatty alcohol-ethylene oxide condensation product used as a protective colloid) and  
2 cc. of acetic acid 50% aqueous solution. Sufficient water was added to give a total volume of 133 cc.

The padding was conducted in a glass beaker.

The muslin was skinned (passed through the atmosphere) for a few seconds and then aged in neutral steam at atmospheric pressure for 20 seconds. A deep, rich blue coloration was obtained having excellent wash-, light- and chlorine-fastness without the minutest evidence of copper precipitation on the fibre.

#### Example II

Example I was repeated with the exception that the Naphthol AS in the padding solution was replaced by 2 grams of phenyl methyl pyrazolone. A tan coloration was produced showing excellent light-, wash- and chlo-

rine-fastness without any perceivable trace of copper precipitation on the fibre.

#### Example III

Example I was repeated with the exception that the Naphthol AS was replaced by an equivalent amount of 2-hydroxybenzeneazo-4-resorcinol and the o-dianisidine, tetrazotized and stabilized with zinc chloride, was replaced by an equivalent amount of zinc chloride double salt of diazotized 5-chloro-o-anisidine. A brown dyeing was obtained which showed excellent light-, wash- and chlorine-fastness with no precipitation of metallic copper on the fibre.

#### Example IV

Example I was again repeated with the exception that the Naphthol AS was replaced by an equivalent amount of 3-hydroxy-2-naphthoic acid o-toluidide and the o-dianisidine, tetrazotized and stabilized with zinc chloride, was replaced by an equivalent amount of zinc chloride double salt of the diazo from 5-n-butyl-sulfamyl-o-anisidine. A red dyeing was obtained which showed excellent light-, wash- and chlorine-fastness with no evidence whatsoever of copper precipitation on the fibre.

#### Example V

A metallizing solution was prepared as follows:

##### Copper solution—

100 grams of tartaric acid  
460 grams of water  
100 grams of copper chloride  
300 cc. of caustic soda 34° Bé.

After formation of a blue solution, 40 grams of sodium chromate anhydrous was added.

3 grams of 3-hydroxy-2-naphthanolide and 1 gram of bis (acetoacet)-o-toluidide were dissolved in 100 cc. of boiling water containing 4.5 cc. caustic soda 34° Bé. To this solution, cooled to about 140° F., was added 10 cc. of the above copper solution.

A 10 gram sample of cotton was padded with the above solution and dried. It was then padded with a solution made by dissolving 8½ grams of zinc chloride double salt of tetrazotized o-dianisidine, 0.5 cc. of a 40% solution of Diazopon AN solution, 13 cc. of 50% aqueous acetic acid solution and water added to make up a total volume of 133 cc., followed by treatment with steam for 25 seconds. A deep jet black dyeing was obtained of excellent wash-, light- and chlorine-fastness with no evidence of deposition of metallic copper on the cotton fibre.

#### Example VI

Example I was repeated with the exception that 10 cc. of the copper solution described therein was replaced by an equivalent volume of the following copper solution:

50 grams of glycine  
400 grams of water  
100 grams of copper chloride  
300 cc. of caustic soda 34° Bé.  
100 grams of sodium perborate

#### Example VII

Example I was repeated with the exception that 10 cc. of the copper solution was replaced by an equivalent volume of the following copper solution:

65 100 grams of glutamic acid  
400 grams of water  
100 grams of copper sulfate  
300 grams of caustic soda 34° Bé.  
70 100 grams of m-nitrobenzenesulfonic acid Na salt

#### Example VIII

A solution was prepared from 120 grams of a commercially available Rapidogen, consisting of 11 grams of o-dianisidine tetrazotized and stabilized with methyl

taurine, 11 grams of 3-hydroxy-2-naphthaniide, 10 grams of sodium hydroxide (100%), 80 grams of combined water and solvents and 50 grams of the copper solution prepared as in Example I. 17 parts of the solution was thickened with 70 parts of starch tragacanth and adjusted with 13 parts of water.

A 10 gram sample of cotton was printed with the paste, steamed in acid steam in a normal manner for 2 minutes, rinsed and dried. The blue dyeing obtained showed excellent light-, wash- and chlorine-fastness with no evidence of metallic copper on the printed cotton fibre.

#### Example IX

A printing paste was prepared as follows:

4 grams of a Rapidogen mix, consisting of equivalent amounts of cresidine diazotized and stabilized with sarcosine, and 3-hydroxy-3'-nitro-2-naphthaniide, 4 cc. of ethylene glycol monoethyl ether, 24 cc. of water, 3 cc. of sodium hydroxide 34° Bé, and 5 cc. of copper solution of Example I were combined and 70 grams of gum tragacanth added to printing thickness.

A 10 gram sample of cotton cloth was printed with the above paste and developed for 2 minutes in acidified steam. The bordeaux dyeing obtained showed excellent light-, wash- and chlorine-fastness with no evidence of metallic copper on the printed cotton fibre.

#### Example X

Example IX was repeated with the exception that 4 grams of the Rapidogen mix was replaced by 4 grams of a Rapidogen mix consisting of an equivalent amount of o-dianisidine tetrazotized and stabilized with methyl taurine, and phenyl methyl pyrazolone and 10 cc. of copper solution of Example I. A tan coloration was produced which showed excellent light-, wash- and chlorine-fastness with no evidence of metallic copper on the printed cotton fibre.

#### Example XI

Example IX was again repeated with the exception that 4 grams of the Rapidogen mix was replaced by 4 grams of a Rapidogen mix consisting of an equivalent amount of 4-benzoylamino-2-methoxy-5-methylaniline diazotized and stabilized with sarcosine, and 3-hydroxy-2-naphthaniide. A violet shade somewhat redder than usual was produced having excellent light-, wash- and chlorine-fastness with no evidence of metallic copper on the printed cotton fibre.

I claim:

1. The process of producing metallized azoic prints and dyeings in situ which comprises treating a cellulosic fibrous material selected from the class consisting of cotton and regenerated cellulose with an azoic coupling component devoid of solubilizing groups and a diazo component derived from an amine base devoid of solubilizing groups to yield an azoic dye component capable of yielding an o,o'-dihydroxy azo configuration at elevated temperatures in the presence of a coordinating agent selected from the class consisting of lower alkylamines and aliphatic amino- and hydroxy-carboxylic acids, and a metallizing copper compound consisting of soluble and dispersible salts and hydroxides of copper, and an oxidizing agent equivalent to 10-100% based on the weight of the metallizing agent, selected from the class consisting of alkali perborates, alkali chromates, hydrogen peroxide, alkali peroxides and nitrobenzenesulfonic acids and their alkali salts.

2. The process according to claim 1 wherein the oxidizing agent is sodium chromate.

3. The process according to claim 1 wherein the oxidizing agent is sodium perborate.

4. The process according to claim 1 wherein the oxidizing agent is m-nitrobenzenesulfonic acid.

5. The process according to claim 1 wherein the oxidizing agent is potassium chromate.

6. The process of producing metallized azoic prints and dyeings in situ which comprises impregnating a cellulosic fibrous material selected from the class consisting of cotton and regenerated cellulose with an azoic coupling component devoid of solubilizing groups at a pH of more than 7 followed by treatment with a diazonium compound derived from an amine base devoid of solubilizing groups, and which azoic component is capable of yielding an o,o'-dihydroxy azo dye configuration in the final dye, followed by treatment at elevated temperatures in the presence of a coordinating agent selected from the class consisting of lower alkylamines and aliphatic amino- and hydroxy-carboxylic acids, and a metallizing copper compound consisting of soluble and dispersible salts and hydroxides of copper, and an oxidizing agent equivalent to 10-100% based on the weight of the metallizing agent, selected from the class consisting of alkali perborates, alkali chromates, hydrogen peroxide, alkali peroxides and nitrobenzenesulfonic acids and their alkali salts.

10 7. The process of producing metallized azoic prints, in situ which comprises printing a cellulosic fibrous material selected from the class consisting of cotton and regenerated cellulose with an alkaline paste consisting of an azoic coupling component devoid of solubilizing groups and a diazoamino compound derived from an amine base devoid of solubilizing groups, which has been diazotized and stabilized with a primary and secondary amine which contains at least one solubilizing

15 group, and which azoic dye component is capable of yielding an o,o'-dihydroxy azo dye configuration in the final dye, followed by treatment with acidified steam in the presence of a coordinating agent selected from the class consisting of lower alkylamines and aliphatic

20 amino- and hydroxy-carboxylic acids, and a metallizing copper compound consisting of soluble and dispersible salts and hydroxides of copper, and an oxidizing agent equivalent to 10-100% based on the weight of the metallizing agent, selected from the class consisting of alkali perborates, alkali chromates, hydrogen peroxide alkali peroxides and nitrobenzenesulfonic acids and their alkali salts.

25 8. A composition of matter for use in azoic dye manufacture which comprises an azoic coupling component devoid of solubilizing groups, a coordinating agent selected from the class consisting of lower alkylamines and aliphatic amino- and hydroxy-carboxylic acids, a metallizing copper compound consisting of soluble and dispersible salts and hydroxides of copper, and an oxidizing agent equivalent to 10-100% based on the weight of the metallizing agent, selected from the class consisting of alkali perborates, alkali chromates, hydrogen peroxide alkali peroxides and nitrobenzenesulfonic acids and their alkali salts in an alkaline solution.

30 9. A composition of matter for use in azoic dye manufacture which comprises an azoic coupling component devoid of solubilizing groups, triethanolamine, copper sulfate and an oxidizing agent equivalent to 10-100% based on the weight of the metallizing agent, selected from the class consisting of alkali perborates, alkali chromates, hydrogen peroxide, alkali peroxides and nitrobenzenesulfonic acids and their alkali salts in an alkaline solution.

35 10. A composition according to claim 9 wherein the oxidizing agent is sodium chromate.

11. A composition according to claim 9 wherein the oxidizing agent is potassium chromate.

12. A composition according to claim 9 wherein the coupling component is Naphthol AS.

13. A composition of matter for use in azoic printing which comprises an azoic coupling component devoid of solubilizing groups, a diazoamino compound derived from an amine base devoid of solubilizing groups which has been diazotized and stabilized with a primary and secondary amine containing at least one solubilizing

group, which azoic dye components are capable of yielding an o,o'-dihydroxy azo dye configuration in the final dye, a coordinating agent selected from the class consisting of lower alkylolamines and aliphatic amino- and hydroxy-carboxylic acids, and a metallizing copper compound consisting of soluble and dispersible salts and hydroxides of copper, and an oxidizing agent equivalent to 10-100% based on the weight of the metallizing agent, selected from the class consisting of alkali perborates, alkali chromates, hydrogen peroxide, alkali peroxides and nitrobenzenesulfonic acids and their alkali salts, in an alkaline medium.

14. A composition of matter for use in azoic printing which comprises an azoic coupling component devoid of solubilizing groups, a diazoamino compound derived from an amine base devoid of solubilizing groups which has been diazotized and stabilized with a primary and secondary amine containing at least one solubilizing group, which azoic dye components are capable of yielding an o,o'-dihydroxy azo dye configuration in the final dye, triethanolamine, copper sulfate and an oxidizing

5

10

15

agent equivalent to 10-100% based on the weight of the metallizing agent, selected from the class consisting of alkali perborates, alkali chromates, hydrogen peroxide, alkali peroxides and nitrobenzenesulfonic acids and their alkali salts, in an alkaline medium.

15. The composition according to claim 14 wherein the oxidizing agent is sodium chromate.

16. The composition according to claim 14 wherein the diazo is dianisidine tetrazotized and stabilized with methyl taurine, and the coupling component is Naphthol AS.

17. The composition according to claim 14 wherein the diazo is 4-benzoylamino-2-methoxy-5-methylaniline diazotized and stabilized with sarcosine, and the coupling component is Naphthol AS.

## References Cited in the file of this patent

## FOREIGN PATENTS

|    |         |               |       |              |
|----|---------|---------------|-------|--------------|
| 20 | 502,144 | Great Britain | ----- | Mar. 7, 1939 |
|    | 531,470 | Great Britain | ----- | Jan. 6, 1941 |